

# UNITED STATES PATENT OFFICE.

FEDERICO GIOLITTI, OF TURIN, ITALY, ASSIGNOR TO SOCIETÀ ANONIMA ITALIANA  
GIO, ANSALDO & C., OF GENOA, ITALY.

## HEAT TREATMENT OF CASTINGS OF SPECIAL STEELS.

1,279,533.

Specification of Letters Patent. Patented Sept. 24, 1918.

No Drawing.

Application filed June 4, 1917. Serial No. 172,570.

To all whom it may concern:

Be it known that I, FEDERICO GIOLITTI, professor of chemistry, a subject of the King of Italy, residing at Turin, Italy (whose post-office address is No. 75 Stradale Moncalieri,) have invented certain new and useful Heat Treatment of Castings of Special Steels, of which the following is a specification.

10. The process forming the object of this invention consists of a special heat treatment to be applied to castings made of special steels belonging to that well-known class of these metals which comprise steels possessing strong thermic hysteresis and characterized by the great frequency of the centers of secondary crystallizations.

20. Steels of the character mentioned form a very vast class comprising steels of widely varying composition, so that it would not be possible to name them all separately.

25. The class of steels in question is, however, well-known and perfectly defined by the above mentioned characteristics; nor can it 30 any doubt arise as to whether any steel of a determined composition belongs to said class or not.

35. The heat treatment forming the object of the invention consists chiefly of the following operations to be applied in the order stated to the casting made of a special steel having the characteristics above mentioned:

40. 1. The steel casting, carefully cleansed and the scale removed, is submitted first to a heat of about 800° C. followed by slow cooling in the furnace. This first operation is performed with the principal object of eliminating the internal tension of the steel. It does not play an absolutely essential part in 45 the attainment of the final mechanical properties which it is desired to impart to the steel by means of the complexive heat treatment, and can sometimes be omitted without any drawback to the final result. This may be very conveniently omitted, though only for economical reasons in treating certain types of steel; and especially for those containing a high percentage of carbon and manganese. As to whether this omission is 50 advisable or not, practical experience will be a sufficient guide in each particular case.

2. The casting is brought gradually—as

well as uniformly in all its parts—to a temperature comprised between a minimum corresponding to about 100° C. above its last 55 point of transformation by heating ( $Ac_3$ ) and a maximum corresponding to about 200° C. above the same point  $Ac_3$ . Such temperature is maintained within the limits above indicated for a length of time which 60 varies greatly with the variation of the dimensions (and above all of the thicknesses), of the pieces treated. Thus, for pieces weighing only a few kilos having thicknesses of about a centimeter, the time in question 65 may be less than half an hour, while for pieces weighing several tons with a thickness of about a decimeter, it may be necessary to prolong the space of time to 10 or 12 hours.

3. The temperature of the piece is allowed to fall slowly and uniformly (in the same furnace) until it reaches 100° to 150° C. higher than the highest point of transformation to the cooling of the treated steel ( $Ar_3$ ). 75 For certain steels of the class in question it may happen that this last interval of temperature covers in part that specified in No. 2.

4. When the piece has reached—uniformly in all its parts—the temperature above mentioned, it is removed from the furnace and submitted to the most rapid cooling possible; compatible with the necessity of preventing cracks.

50. This last condition depends, as is well known on the composition of the steel, on the way in which the piece has been cast and on the dimensions and form of the piece itself.

55. The cooling medium will thus have to be selected according to the above conditions of facts following the well known practical rules.

60. Thus, pieces of simple form and of relatively small dimensions formed of steel of average hardness will be left to cool in a 65 current of cold air either natural or produced artificially.

65. The large pieces of a very complicated form or with thin parts and formed of hard steels, will be left to cool in a closed space. 100 The small pieces or those of simple form and those formed of steel with a small percentage of carbon, of manganese and of chromium, may be cooled by immersing them

in molten lead at just above its melting point, or in hot or cold oil, or in hot water.

5. The piece treated as above is submitted to a uniform annealing.

5. The temperature at which this annealing should be carried out depends on the final mechanical properties (particularly the ultimate resistance and the elastic limit) which are desired in the material of the piece submitted to treatment. The conditions of this annealing (above all as regards time and temperature) will, thus be determined for each particular case for each type of steel, by means of some preliminary tests made on 10 the material submitted to the above mentioned treatment and followed by mechanical tests.

In case the treatment by the first four steps (paragraphs 1, 2, 3 and 4) produces a 20 product having the desired elastic limit, the annealing step may be omitted.

It is, however, always advisable (and especially when a product of great tenacity and resiliency is wanted) to choose the material and to perform the treatment in such a way that the elastic limit of the steel after the treatment described in No. 4 will be above the required value so as to finally bring this down to the desired point by 30 efficient annealing.

It may happen in some cases, that practical experience will show that it is advisable to repeat twice or more, one, or even several of the treatments described in the five preceding 35 paragraphs.

The application of the whole of the operations above described, (performed under the prescribed conditions and in the order indicated) to steels having the characteristic 40 properties specified at the beginning of this specification, permits one to obtain the following results, the novelty and technical importance of which are in themselves apparent:

45 A. Increase of the tenacity and resiliency of the steel simply cast to the approximate values, and sometimes also greater than those which it is generally possible to obtain only in forged and treated steels. 50 Such results appear above all evident in the endurance and bending tests.

B. The attainment of the values of the elastic limit and reduction of area before breaking, under tensile stress, such as are 55 generally attained only with forged and treated steels.

60 C. Total elimination of the characteristic crystalline structure of the cast steels. Such structure, always a sign of fragility, is substituted (in the above mentioned steels submitted to the described treatment) by a fibrous structure similar to that which is characteristic of forged steels.

In order to be entirely clear, as to the

steels treated, the following three examples 65 may be cited:

*Example I.—Composition of the steel.*

|            |       |    |
|------------|-------|----|
| Carbon     | 0.18% | 70 |
| Silicon    | 0.25% |    |
| Manganese  | 0.90% |    |
| Nickel     | 0.80% |    |
| Chromium   | 0.40% |    |
| Titanium   | 0.30% |    |
| Molybdenum | 0.20% | 75 |

(1) The first heating and cooling (first step of the process) is not necessary with this type of steel.

(2) The highest temperature for the combination in the second step of the thermic treatment is 950° C.

(3) The heating in the third step must be maintained at about 720° C.

(4) The cooling (in the fourth step) is effected in a current of cooled air.

(5) The annealing is effected at 500° C.

*Example II.—Composition of the steel.*

|           |       |    |
|-----------|-------|----|
| Carbon    | 0.09% | 90 |
| Silicon   | 0.25% |    |
| Manganese | 0.70% |    |
| Nickel    | 1.00% |    |
| Vanadium  | 0.28% |    |

For this steel:

(1) The first heating (first step of the process) must be to a temperature of about 800° C., with this type of steel.

(2) The highest temperature for the combination in the second step of the thermic treatment is 1000° C.

(3) The heating in the third step must be maintained at about 800° C.

(4) The cooling (in the fourth step) is best done in oil at 90° C.

(5) Annealing is not necessary.

*Example III.—Composition of the steel.*

|            |       |     |
|------------|-------|-----|
| Carbon     | 0.47% | 110 |
| Silicon    | 0.20% |     |
| Manganese  | 0.75% |     |
| Chromium   | 1.70% |     |
| Vanadium   | 0.30% |     |
| Molybdenum | 0.20% |     |

For this steel:

(1) The first heating (first step) must be to about 800° C., with this type of steel.

(2) The highest temperature for the combination in the second step of the thermic treatment is 850° C.

(3) The heating in the third step must be maintained at about 680° C.

(4) The cooling (in the fourth step) is made in the atmospheric air in an inclosed space.

(5) The annealing is performed at 550° C.

The position of point  $A_c$ , for a casting of a given steel varies considerably with the

condition of homogeneity that said steel presents immediately after the step of casting and the following solidification. Also such condition of homogeneity varies considerably with the varying temperature of the melted steel during the casting step and with the nature of the material forming the molds in which the steel is cast. (Cast iron molds, dry sand molds, moist sand molds, etc.)

The point  $Ar_3$  cannot be absolutely and precisely determined, since corresponding to it, the determining transformation curve of the steel, that serves to determine it shows a well graduated deformation not perfectly localized. From this it follows that the determination of point  $Ar_3$ , according to the steel constitution, may only be obtained in an approximation of about  $50^{\circ}$  C. In practice, the position of this point then is determined more precisely by means of few heat treatment tests.

Further the position of both the points  $Ac_3$  and  $Ar_3$ , but more particularly of the point  $Ar_3$ —especially depends upon the speed of cooling of the casting under treatment, said speed greatly modifying the importance of the heat-hysteresis phenomenon, which may produce—as is well known—great variations in the transformation points. From this, it follows, that the positions of such points also greatly depend upon the size and shape of the castings under treatment.

This said,—in order not to give an abso-

lute value to the hereinafter referred figures—the approximate limits, are here indicated between which the positions of points  $Ac_3$  and  $Ar_3$  for each of the three examples given above, may vary according to conditions which may be easily realized in practice:—

Example I— $Ac_3=780^{\circ}$  to  $850^{\circ}$  C.  
 $Ar_3=580^{\circ}$  to  $650^{\circ}$  C.

Example II— $Ac_3=820^{\circ}$  to  $900^{\circ}$  C.  
 $Ar_3=600^{\circ}$  to  $700^{\circ}$  C.

Example III— $Ac_3=730^{\circ}$  to  $800^{\circ}$  C.  
 $Ar_3=600^{\circ}$  to  $650^{\circ}$  C.

I claim:

1. A process of treating cast steels having strong thermic hysteresis, which comprises slowly heating the steel to a temperature of about  $100^{\circ}$  C. to  $200^{\circ}$  C. above the point  $Ac_3$  and maintaining the said steel at said temperature for a time, then cooling slowly to a temperature of about  $100$  to  $150^{\circ}$  C. above the point  $Ar_3$ , and then rapidly cooling the steel so treated.

2. The process of claim 1, preceded by the steps of heating to about  $800^{\circ}$  C. and then slowly cooling.

3. The process of claim 1, followed by an annealing operation.

In witness whereof I have hereunto signed my name in the presence of two witnesses.

FEDERICO GIOLITTI.

Witnesses:

G. B. ZAMARDO,  
 WILLIS E. RUFFNER.